

## UNITED STATES PATENT OFFICE.

CHARLES F. KETTERING AND THOMAS MIDGLEY, JR., OF DAYTON, OHIO, ASSIGNEES,  
BY MESNE ASSIGNMENTS, TO GENERAL MOTORS CORPORATION, OF DETROIT, MICH-  
IGAN, A CORPORATION OF DELAWARE.

## METHOD AND MEANS FOR USING LOW-COMPRESSION FUELS.

No Drawing.

Application filed January 3, 1924. Serial No. 684,255.

This invention relates to the art of suppressing a fuel knock when a combustible gaseous mixture containing a low compression fuel such, for example, as kerosene and gasoline are burned under a relatively high pressure. The principal objects of this invention are to employ iodine compounds to suppress the fuel knock.

This application is a continuation in part 10 of our copending application, Serial No. 553,040, filed April 15, 1922.

Kerosene has a critical compression pressure of about 55 pounds. The critical compression pressure of gasoline varies from 15 about 75 pounds for the commoner forms now marketed to about 125 pounds for "aviation gasoline" employed in airplane engines. These fuels are termed low compression fuels. When the vapors of any one 20 of them is mixed with air, compressed to a compression pressure in excess of the normal critical compression pressure of the fuel, and burned, as in an internal combustion engine, a fuel knock is produced.

25 We have found that vapors of iodine compounds added to the fuel-air mixture suppress this fuel knock and permit an increase in the engine compression pressure with a normal burning characteristic of the fuel.

30 By way of an example of one method of carrying out our invention, we dissolve ethyl iodide in gasoline having a normal critical compression pressure of about 75 pounds, to form a fuel consisting by volume 35 of 5% ethyl iodide and 95% gasoline. This solution or high compression fuel is fed through a carburetor into the cylinder of an internal combustion engine having a compression pressure of about 100 pounds, 40 the solution being vaporized and mixed with air as is common practice in engine opera-

tion. The gaseous high compression fuel is ignited and the engine operated without a fuel knock. The gasoline forms the fuel base and the iodine compound increases the 45 critical compression pressure of this base.

This process may be varied by changing the proportions according to the increase in critical compression pressure desired and by using other iodine compounds in place 50 of the ethyl iodide. Among the substances which may be employed are other alkyl compounds including amyl, methyl and propyl iodide, potassium iodide, phenyl iodide, iodoform, tin tetraiodide, lead diethyl diiodide, lead diphenyl di-iodide and elemental iodine.

We prefer to employ the iodine compounds which are soluble in the fuel to promote the mixing of the two. Blending 60 agents may be employed if the iodine compound does not dissolve readily in the fuel. The compound may be added to the fuel air mixture just before the latter is burned.

65 What is claimed is as follows:

1. A fuel for internal combustion engines, containing iodine.

2. A composition of matter comprising a low compression fuel, such as kerosene or gasoline; and an alkyl compound of iodine 70 incorporated homogeneously therein and adapted to increase the critical compression pressure of the fuel.

3. A composition of matter comprising a low compression fuel; and an ethyl compound of iodine incorporated therein. 75

4. A composition of matter comprising gasoline; and ethyl iodide.

In testimony whereof we hereto affix our signatures.

CHARLES F. KETTERING.  
THOMAS MIDGLEY, JR.